

April 18, 1939.

I. E. ASKE

2,154,717

CYLINDER HEAD

Filed June 22, 1936

FIG. 1.



FIG. 2.



INVENTOR  
IRVING E. ASKE  
BY  
Leverance & Van Antwerp  
ATTORNEYS

## UNITED STATES PATENT OFFICE

2,154,717

## CYLINDER HEAD

Irving E. Aske, Muskegon, Mich., assignor to  
 Campbell, Wyant & Cannon Foundry Company, Muskegon Heights, Mich., a corporation  
 of Michigan

Application June 22, 1936, Serial No. 86,529

3 Claims. (Cl. 123—191)

This invention relates to improvements in the heads or covers which are located over the ends of the cylinder blocks of internal combustion engines.

Such cylinder heads ordinarily heretofore have been made from cast iron, and the parts at the lower side of the head which are over the ends of the engine cylinders and around and over the intake and exhaust valve ports have required machining to produce a smooth surface. Cast iron as a material for engine cylinder blocks and covering heads is a very satisfactory material but the parts exposed to the gaseous fuel which is burnt or exploded are susceptible to the collection of carbon such as is produced in internal combustion engines due to the incomplete burning of the fuel. The cast iron is a very good conductor of heat from the cylinder walls and combustion chamber to the water which is located in certain passages or cavities in the cylinder head. The necessity of rapid conduction of heat in order that the engine parts may not overheat is obvious.

In my invention it is a primary object and purpose to produce a cylinder cover for the cylinders and laterally connected combustion chambers therefor which will be smooth and not require machining after casting, to which carbon does not normally adhere, and in which there is the same rapidity of heat conduction as in an engine head made wholly from cast iron. Specifically it is an object and purpose of the present invention to produce a cover or head for the cylinder block of cast iron lined with steel at its underside at each cylinder and combustion chamber associated with the cylinder, the engaging surfaces of the steel liners and of the cast iron being fused together to provide the desired rapid conduction of heat which is generated in the engine operation. The engine cover or head is produced by placing in the mold the several steel members which serve as liners, one for each cylinder of the engine and the combustion chamber connected therewith, the steel liners being properly pre-formed into shape, and then pouring molten iron into the mold and at a temperature sufficiently high that, with the quantity of molten iron used and the retention of high temperature in the iron for a considerable period of time after the iron is poured, there is produced a substantially integral joint of the steel liners to the cast iron cylinder head over the entire engaging surfaces of the two ferrous materials, thereby obtaining in effect an integral product having the same

degree of heat conduction as all-cast cylinder heads or covers.

The invention will be understood from the following description, taken in connection with the accompanying drawing, in which,

Fig. 1 is an underplan view of the cylinder block cover or head showing the liner for one cylinder and combustion chamber, and

Fig. 2 is a fragmentary transverse vertical section through the upper part of an engine illustrating a cylinder and combustion chamber therefor having my invention applied.

Like reference characters refer to like parts in the figures of the drawing.

The engine block 1 is of usual construction having vertical cylinders 2, ports 3, opened and closed by valves 4 in the usual manner, the cylinder block having a desired number of cylinders and being of a cast iron material. The head or cover 5 is principally of cast iron, carrying the usual spark-plugs 6, the inner ends of which extend one to each of the combustion chambers 7. There is a combustion chamber between the port entrance and the upper end of each cylinder 2 as shown in Fig. 2.

With my invention a sheet metal liner is provided having an upper side 8 and with downwardly extending flanges 9 to line the combustion chamber 7, and thence extended farther in a section 10 to line the underside of the head over the upper end of each of the cylinders. The shape of the sections 10 will correspond to the shape of the upper end of the pistons 11 which are mounted in the cylinders. In Fig. 2 the upper end of the cylinder is of a convex form and the part 10 is similarly shaped so as to be spaced a short distance from the convex upper end of the piston at all points beyond the combustion chamber, which combustion chamber extends partly over the upper end of the piston as shown.

The liner is of steel having a carbon content preferably as high as can be practically used in die stamping and forming operations, that is, the carbon content cannot be too high or much beyond .20% as it will lack ductility so that it cannot be properly drawn cold. The liners, one for each cylinder and combustion chamber in the engine, are properly placed in the mold and the molten iron is poured into the mold contacting the liner at all surfaces opposite the positions of the combustion chambers and cylinders. The molten metal is at a high degree of temperature, for example, at least 2500° or 2600° F. preferably. With the body of molten metal used and the escape of heat retarded and checked by the mold,

at such initial pouring temperatures substantially complete fusion of the steel liners with the cast iron material of the rest of the head is attained.

- 5 From the foregoing it is evident that when the completed cast head is taken from the mold there will be presented smooth surfaces at the inner sides of the steel liners and no machining of such surfaces is required to finish them to proper shape.
- 10 Steel does not have carbon adhere thereto so that the steel surfaces over the combustion chambers and the pistons remain clean and free of carbon collection. The fusion joinder of the liners to the cast iron cover provides the same
- 15 high degree of conductivity of heat to the cooling water as does a solid cast iron head or cover.

The invention is very practical, simple to produce and particularly useful in operation. The claims appended hereto define the invention.

I claim:

1. A cast iron cover or head for cylinder blocks of internal combustion engines and a steel lining at the inner side of said head over the cylinders and combustion chambers, said lining and cast iron head having fused connection.

2. A cast iron cylinder head or cover for internal combustion engines and a preformed steel lining member at the inner side of said head fused thereto, adapted to provide the upper wall of a combustion chamber connected with the cylinder in the engine to which the head or cover is applied.

3. A cylinder head structure comprising a cylinder cover member of cast iron and a sheet steel member having formed therein a combustion chamber, the said members having a fused connection throughout their opposed areas.

IRVING E. ASKE.